# EUROPEAN PATENT SPECIFICATION

(11) **EP 0 017 072 B1**
(45) Date of publication and mention of the grant of the patent: **06.07.1983**
(21) Application number: 80101408.5
(22) Date of filing: 18.03.1980
(51) Int. Cl.: C10M 3/20, C10M 3/22

(54) **Water-resistant lubricant for compressors and marine engines**
Wasserwiderstandsfähiges Schmiermittel für Kompressoren und Schiffsmotoren
Lubrifiant résistant à l'eau pour compresseurs et moteurs marins

(30) Priority: 02.04.1979 US 26269
(43) Date of publication of application: 15.10.1980
(73) Proprietor: THE DOW CHEMICAL COMPANY, Midland Michigan 48640-1967 (US)
(72) Inventor: Carswell, Robert, Lake Jackson Texas (US); McGraw, Philip Wayne, Lake Jackson, County of Brazoria, Texas (US)
(74) Representative: Casalonga, Alain

## Description

This invention relates to water-resistant lubricants for compressors and marine engines, especially for use in rotary screw compressors.

Rotary screw air compressors are well-known in the art as can be seen from US-A-3,073,513, issued to Bailey, January 15, 1963.

It is well-known to use hydrocarbon lubricating oils to seal the rotors of the foregoing rotary screw air compressors, lubricate the bearing and cool the compressed gases. Due to the high temperature and pressure of the air, it has been found that these hydrocarbon oils break down and create a sludge in a relatively short time, i.e., about 1000 hours or less.

In attempts to increase the intervals between changes of the lubricants, silicone fluids have been used. However, these fluids are very expensive and represent a considerable capital investment because a new compressor unit with different bearings and seals is required.

It is known that synthetic esters made from dicarboxylic acids have been used in an attempt to develop a relatively inexpensive and long- lasting lubricant. However, it has been found that these synthetic esters are not hydrolytically stable, and therefore do not have the long life required for use in air compressors.

Synthetic lubricants comprising a major amount of a polyester and a minor amount of a monocapped polyglycol are known from GB-A-1,162,818, I.C.I., August, 1969. GB-A-9 21238 relates to lubricating compositions based on neutral carboxylic esters and a small proportion of alkoxyamines. These compositions may also contain 1 to 40% of polyoxyalkylene glycolethers. However, these compositions are disclosed to be only useful in aircraft gas turbines where gross contamination with water is not a problem.

It now has been found that a suitably inhibited blend of hindered alkanoic esters of aliphatic polyhydric alcohols having 3 to 6 hydroxyl groups and 5 to 10 carbon atoms with polyoxyalkylene glycols and their mono or dialkyl ethers has the required high temperature viscosity and stability to oxygen and water.

The present invention relates to a water resistant base lubricant composition for compressor and marine engines which is characterized in that it contains
(A) 15 to 45 weight percent of an ester of a hindered polyhydric alcohol having 3 to 6 hydroxyl groups and from 5 to 10 carbon atoms with one or more alkanoic acids having 4 to 18 carbon atoms, and
(B) 85 to 55 weight percent of one or more compositions having a flash point greater than 191 °C and having the formula where R is hydrogen or an alkyl group of 1-6 carbon atoms, R' is hydrogen or methyl, and n is a number having an average value which will give a molecular weight range from 400 to 5000.

An additional aspect of the present invention comprises the above base lubricant with the addition of effective amounts of oxidation inhibitors, corrosion inhibitors, and metal or copper deactivators.

While the lubricants of this invention are useful in a rotary screw, sliding vane, and reciprocation piston compressors, they are also useful in other mechanical devices where hydrolytic stability is desired or necessary such as outboard motors or marine engines in general.

The neutral esters used in this invention are commercially available. Examples of suitable hindered esters are esters of trimethylol ethane with alkanoic acids of 4-18 carbon atoms, esters of trimethylol propane with alkanoic acids of 4-18 carbon atoms, esters of trimethylol butane with alkanoic acids of 4-18 carbon atoms, and esters of pentaerythritol or dipentaerythritol with alkanoic acids of 4-18 carbon atoms.

Specific examples of these esters are trimethylolethane tricaproate, trimethylolpropane trivalerate, trimethylolpropane tri n-heptanoate, trimethylolpropane tripelargonate, trimethylolpropane tricaprate, pentaerythritol tetra- caproate, dipentaerythritol hexabutyrate, pentaerythritol tetrastearate and the related esters with mixed acid moieties.

Examples of the polyoxyalkylene glycols used in this invention are those derived from ethylene, propylene, 1-2, or 2-3 butylene oxide. The above oxides may be polymerized alone in combination. The combined oxides may also be combined in a random or block addition. While some of the above compounds may be of a hydrophylic nature, those of a hydrophobic nature are preferred, such as those derived from propylene oxide, butylene oxides or combinations thereof.

Examples of suitable capped polyoxyalkylene glycols are those derived from ethylene, propylene, and butylene oxides wherein the alkylene oxides are initiated from monofunctional alkanols having 1-6 carbon atoms in a known manner. The above monoalkyl ethers of polyoxyalkylene glycols can be further modified in a known manner to give the dialkyl ethers.

The foregoing glycols should have a flash point greater than 191°Cand preferably greater than 232°C. They also should have a number average molecular weight range from about 400 to 5000 and preferably in the range 700 to 2500.

The foregoing esters and glycols are blended to give a base lubricant composition containing 15 to 45 weight percent of the esters and 85 to 55 weight percent of the glycol with the ranges 22 to 35 and 78 to 65 being the preferred ranges, respectively.

The compositions of this invention are selected so as to have a viscosity in the range of 5-25x10-⁶ m²/s (5 to 25 centistokes) at 99°C and preferably 6-16 x 1 0 -6 m²/s (6 to 16 centistokes) at 99°C and a pour point in the range of -17.8° to -54°C.

The final lubricant compositions of this invention contain effective amounts of conventional anti-oxidants, corrosion inhibitors and metal or copper deactivators.

Examples of useful antioxidants which can be used herein are phenyl naphthylamines, i.e., both alpha- and beta-naphthyl amines, diphenyl, amine, iminodibenzyl, p,p'-dioctyl-diphenylamine, and related aromatic amines. Other suitable antioxidants are hindered phenolics such as 6-t-butyl phenol, 2,6-di-t-butyl phenol and 4-methyl-2,6-di-t-butyl phenol.

Examples of suitable corrosion inhibitors are the metal sulfonates such as calcium petroleum sulfonate, barium dinonylnaphthalene sulfonate and basic barium dinonylnaphthalene sulfonate (carbonated or noncarbonated).

Examples of suitable N-heterocyclic metal or copper deactivators are imidazole, benzimidazole, pyrazole, benzotriazole, tolutriazole, 2-methyl benzimidazole, 3,5-dimethyl pyrazole, and methylene bisbenzotriazole.

An effective amount of the foregoing additives is generally in the range from 0.1 to 5.0 percent by weight for the antioxidants, 0.1 to 5.0 percent by weight for the corrosion inhibitors, and 0.001 to 0.5 percent by weight for the metal deactivators, all percentages being based on the total weight of the esters and the glycols. It is to be understood that more or less of the additives may be used depending upon the circumstances for which the final composition is to be used.

The following examples illustrate the invention.

### Example 1

The following composition was prepared.

175 Pounds (79.4 kg) polypropylene glycol (number averge molecular weight 1200), 75 pounds (34.0 Kg) pentaerythritol tetraester of alkanoic acids, 3.75 pounds (1.70 kg) p,p'-dioctyl diphenylamine, 1.25 pounds (0.57 kg) basic barium dinonyl-naphthalene sulfonate in mineral oil, and 0.125 pound (0.28 kg) benzotriazole.

The polyglycol and the ester were weighed into a 30 U.S. gallon (114 I) stainless steel mixing vessel, equipped with a paddle stirrer and a controllable electric heating element. The temperature was raised to 45°-55°C with stirring. The additives were then weighed in, in the order given above.

The above 25 U.S. gallon (94.5 I) mixture was allowed to stir with the heating maintained at 45°-55°C until a clear solution was obtained. A clear light brown solution was obtained and was drained from the mixing vessel by opening a valve situated in the base of the vessel. The blend was collected into 5 U.S. gallon 18.9 I) containers. The fluid was retained for testing as described in the following manner. This example illustrates the preparation of a blend of 70 weight percent polyglycol and 30 weight percent of a polyester.

50 Grams of fluid prepared above was sealed in a rotary bomb and tested for oxidation resistance in accordance with American Society for Testing Materials (ASTM) Test D-2272. The fluid gave 18.5 hours in the oxidation test.

It is to be noted in this example and the following examples that the number of hours in the oxidation test can vary about two hours over and under the given numbers because the test procedure is not exactly reproducible.

300 ml of the above fluid was tested for corrosion resistance in accordance with ASTM Test D-665 (procedure A). The fluid passed the test.

Four and one-half U.S. gallons (17.0 I) of the above fluid was placed in a 100 cubic feet (2.83 m³) per minute rotary screw air compressor and the compressor was run for 6000 continuous hours with periodic shutdowns at 1000-hour intervals to take a 4-ounce (113 g) sample for analysis. Four ounces (113 g) of new fluid replaced the withdrawn sample. The test was terminated at 6000 hours due to a breakdown of the compressor which was not associated with the lubricant. Upon examination the fluid withdrawn from the compressor was found to be in excellent condition. Similar results will be obtained with the corresponding dibutyl ether or butyl ether of polypropylene glycol having a similar molecular weight.

### Example 2

Following the procedures set forth in Example 1, a blend of 76 weight percent of the polypropylene glycol and 24 weight percent of trimethylolpropane tripelargonate was prepared with the same percentages of the additives. This formulation when tested by the above oxidation test gave 16 hours and 50 minutes and passed the corrosion test.

### Example 3

Following the procedures set forth in Example 1 with the same additives, a blend of 80 weight percent of the polypropylene glycol and 20 weight percent of a trimethylolpropane fatty acid ester was prepared. This formulation gave 15 hours and 10 minutes in the above oxidation test and passed the corrosion test.

### Controls 1-3

Following the oxidation test of Example 1, a hydrocarbon lubricant (Control #1 a a petroleum oil (Control #2) and a synthetic fluid based on a dicarboxylic acid ester (Control _{#}3) were tested. The above three lubricants have been recommended for use in rotary screw compressors by lubrication engineers. The results are shown in Table I.

From the foregoing, it is indicated that lubricating oils have a relatively short life span and that while dicarboxylic acid esters are better than lubricating oils they are less effective than the compositions of this invention. Furthermore, the compositions containing trimethylolpropane esters of Example 2 are vastly improved over the known esters of Control 3. Likewise, the compositions containing esters of Example 1 are even more improved over Example 2 and Control 1.

## Claims

1. A water resistant base lubricant composition for compressor and marine engines characterized in that it contains
(A) 15 to 45 weight percent of an ester of a hindered polyhydric alcohol having 3 to 6 hydroxyl groups and from 5 to 10 carbon atoms with one or more alkanoic acids having 4 to 18 carbon atoms, and
(B) 85 to 55 weight percent of one or more compositions having a flash point greater than 191°C and having the formulaa where R is hydrogen or an alkyl group of 1-6 carbon atoms, R' is hydrogen or methyl, and n is a number having an average value which will give a molecular weight range from 400 to 5000.

2. The lubricant composition of claim 1 wherein the hindered polyhydric alcohol is pentaerythritol and the polyoxyalkylene glycols of formula I have a number molecular weight range from 700 to 2500.

3. The lubricant composition of Claim 1 or 2 characterized in that the weight percent of the ester ranges from 22 to 35 and the weight percent of the polyglycol ranges from 78 to 65.

4. The lubricant composition of Claim 2 or 3 wherein the glycol is polypropylene glycol having a number average molecular weight of 1200.

5. The lubricant composition of Claim 4 which comprises 30 weight percent of said ester and 70 weight percent of said polypropylene glycol.

6. Finished lubricant composition containing the base composition of Claim 1 and
(C) an effective amount of an antioxidant,
(D) an effective amount of a ferrous metal corrosion inhibitor, and
(E) an effective amount of a metal deactivator.

7. The composition of Claim 6 characterized in that it contains.
(C) 0.1 to 5.0 weight percent of an aromatic amine antioxidant,
(D) 0.1 to 5.0 weight percent of a metal salt of an aromatic sulfonic acid as corrosion inhibitor, and
(E) 0.001 to 0.5 weight percent of a N-heterocyclic metal deactivator;
the percentages being based on the total weight of the esters and the glycols.

## Revendications

1. Composition lubrifiante de base résistant à l'eau pour compresseurs et moteurs marins, caractérisée par le fait qu'elle contient: (A) 15 à 45% en poids d'un ester d'un alcool polyhydrique, comportant un empêchement stérique, ayant 3 à 6 groupes hydroxyle et de 5 à 10 atomes de carbone, avec un ou plusieurs acides alcanoïques ayant 4 à 18 atomes de carbone, et (B) 85 à 55% en poids d'une ou de plusieurs composition(s) ayant un point d'éclair supérieur à 191°C et ayant la formule: dans laquelle R est de l'hydrogène ou un groupe alkyle ayant 1 à 6 atomes de carbone; R' est de l'hydrogène ou le groupe méthyle, et n est un nombre ayant une valeur moyenne qui donnera un poids moléculaire allant de 400 à 5000.

2. Composition lubrifiante selon la revendication 1, dans laquelle l'alcool polyhydrique comportant un empêchement stérique est le penta-érythritol, et les polyalkylène-glycols de formule (1) ont un poids moléculaire en nombre allant de 700 à 2500.

3. Composition lubrifiante selon les revendications 1 ou 2, caractérisée par le fait que le pourcentage pondéral de l'ester va de 22 à 35 et que le pourcentage pondéral du polyglycol va de 78 à 65.

4. Composition lubrifiante selon les revendications 2 ou 3, dans laquelle le glycol est le polypropylèneglycol ayant un poids moléculaire moyen en nombre de 1200.

5. Composition lubrifiante selon la revendication 4, qui comprend 30% en poids dudit ester et 70% en poids dudit polypropylèneglycol.

6. Composition lubrifiante terminée contenant la composition de base selon la revendication 1 et:
(C) une quantité efficace d'un anti-oxydant
(D) une quantité efficace d'un inhibiteur de corrosion des métaux ferreux, et
(E) une quantité efficace d'un désactiveur de métaux.

7. Composition selon la revendication 6, caractérisée par le fait qu'elle contient:
(C) 0,1 à 5% en poids d'une amine aromatique comme antioxydant
(D) 0,1 à 5% en poids d'un sel métallique d'un acide sulfonique aromatique comme inhibiteur de corrosion, et,
(E) 0,001 à 0,5% en poids d'un désactiveur de métaux N-hétérocyclique;
les pourcentages étant calculés sur le poids total des esters et des glycols.

## Patentansprüche

1. Grundlage für eine wasserfeste Schmiermittelzusammensetzung für Kompressor- und Schiffsmotoren, dadurch gekennzeichnet, dass sie enthält:
(A) 15 bis 45 Gewichtsprozent eines Esters eines gehinderten mehrwertigen Alkohols mit 3 bis 6 Hydroxylgruppen und 5 bis 10 Kohlenstoffatomen, mit einer oder mehreren Alkanosäuren mit 4 bis 18 Kohlenstoffatomen, und
(B) 85 bis 55 Gewichtsprozent einer mehrerer Zusammensetzungen der nachstehenden Formel mit einem Flammpunkt über 191°C: wobei R Wasserstoff oder eine Alkylgruppe mit 1 bis 6 Kohlenstoffatomen, R' Wasserstoff oder Methyl und n eine Zahl mit einem Durchschnittswert ist, die einen Molekulargewichtsbereich von 400 bis 5000 einstellt.

2. Die Schmiermittelzusammensetzung gemäss Anspruch 1, in der es sich bei dem gehinderten mehrwertigen Alkohol um Pentaerythritol handelt und die Polyoxyalkylenglykole der Formel eine Zahl zur Einstellung eines Molekulargewichtsbereichs von 700 bis 2500 haben.

3. Die Schmiermittelzusammensetzung gemäss Anspruch 1 oder 2, dadurch gekennzeichnet, dass der Gewichtsprozentbereich des Esters zwischen 22 und 35 und der Gewichtsprozentbereich des Polyglykols zwischen 78 und 65 liegt.

4. Die Schmiermittelzusammensetzung gemäss Anspruch 2 oder 3, in der es sich bei dem Glykol um Polypropylenglykol mit einem durchschnittlichen Molekulargewicht um 1200 handelt.

5. Schmiermittelzusammensetzung gemäss Anspruch 4, die 30 Gewichtsprozent des genannten Esters und 70 Gewichtsprozent des genannten Polypropylenglykols enthält.

6. Fertige Schmiermittelzusammensetzung, die als Grundlage die Zusammensetzung gemäss Anspruch 1 und
(C) eine ausreichende Menge eines Oxidationsschutzmittels,
(D) eine ausreichende Menge eines Eisenmetall-Korrosionsschutzmittels .und
(E) eine ausreichende Menge eines Metall-Desaktivierungsmittels enthält.

7. Die Zusammensetzung gemäss Anspruch 6, dadurch gekennzeichnet, das sie
(C) 0,1 bis 5,0 Gewichtsprozent eines aromatischen Amin-Oxidationsschutzmittels,
(D) 0,1 bis 5,0 Gewichtsprozent eines Metallsalzes einer aromatischen Sulfonsäure als Korrosionsschutzmittel, und
(E) 0,001 bis 0,5 Gewichtsprozent eines n-heterozyklischen Metall-Desaktivators enthält, wobei sich die Prozentwerte jeweils auf das Gesamtgewicht der Ester und der Glykole beziehen.
